

## UNITED STATES PATENT OFFICE

2,161,576

## SILVER BASE ALLOY

Franz R. Hensel, Kenneth L. Emmert, and James W. Wiggs, Indianapolis, Ind., assignors to P. R. Mallory & Co., Inc., Indianapolis, Ind., a corporation of Delaware

No Drawing. Application April 13, 1939,  
Serial No. 267,607

4 Claims. (Cl. 75—173)

This invention relates to a new silver alloy and is concerned more particularly with an alloy which has improved physical and electrical characteristics.

5 It is one of the objects of the invention to provide a silver base material which can be used for an electrical make and break contact, retaining very low contact resistance, having very low material transfer and being free from welding and sticking under heavy electrical loads.

Another object of the invention is to provide a new silver base alloy which has improved tensile properties and which also shows considerable improvements as far as corrosion resistance is concerned.

Other objects of the invention will be apparent from the following description, taken in connection with the appended claims.

The present invention comprises a combination of elements, methods of manufacture and the products thereof, brought out and exemplified in the disclosure hereinafter set forth, the scope of the invention being indicated in the appended claims.

25 While a preferred embodiment of the invention is described herein, it is contemplated that a considerable variation may be made in the method of procedure and the combination of elements, without departing from the spirit of the invention.

The present invention relates to an alloy of silver, magnesium and thorium. In the formation of the new alloy, it is preferable to provide a composition of the materials specified in the following proportions:

|           | Per cent   |
|-----------|------------|
| Magnesium | .05 to 15  |
| Thorium   | .005 to 10 |
| Silver    | Balance    |

40 It is likewise possible to improve the characteristics of silver alloys containing additional ingredients by the combined addition of magnesium and thorium. Such elements are primarily copper and gold, zinc, cadmium, indium, thallium, zirconium and tin. We have also found that iron group metals may be added up to several percentages, and that the alloys may contain considerable percentages of precious metals, taken from the palladium and platinum group.

45 A preferred range of magnesium is .05 to 8%, because up to that percentage, magnesium is taken up in alpha solution in silver and we have found that silver and magnesium, up to 8%, can be alloyed very readily, and the cast ingots can

be rolled, swaged or drawn into desirable shapes, such as sheet, bar stock, wire, strip and the like. A more specific preferred range for magnesium is 1 to 4%. A preferred range for thorium is 1 to 3%.

5 The addition of thorium to silver magnesium base alloys further improves the physical and electrical characteristics. Thorium has a very high melting point and one of its outstanding properties is the great deoxidizing power, resulting in completely deoxidized and clean silver alloys, which are of advantage particularly in their use as electrical contacting elements, in order to prevent localized build-up. Thorium was introduced in the form of a silver thorium master alloy, having a high concentration of thorium and being prepared by powder metallurgical methods. No difficulty was encountered in absorbing thorium in the silver.

10 We have investigated a series of compositions and have found that the following alloys which are given by way of example have shown very excellent physical properties, and particularly electrical properties, if used in the form of electrical contacts.

|               | Per cent   |
|---------------|------------|
| (1) Magnesium | 3          |
| Thorium       | 2½         |
| Silver        | Balance    |
| (2) Magnesium | 3 30       |
| Thorium       | .25        |
| Silver        | Balance    |
| (3) Magnesium | 6          |
| Thorium       | 1½         |
| Silver        | Balance 35 |

These ingredients in the proportions named above, are melted together and poured into a suitable mold. It was pointed out above that it was found desirable to add the thorium in the form of silver-thorium master alloy. It was also found desirable to add the magnesium in the form of a silver-magnesium master alloy, of high magnesium concentration. Master alloys of this type have a lower melting point and therefore will go readily into the silver melt. Since silver-magnesium has a tendency to deoxidize and form a dross, it has been found desirable to melt such alloys either in a reducing atmosphere or use suitable fluxes which cover the melt.

40 The addition of magnesium in the form of a master alloy has also reduced the loss of magnesium and therefore has made it possible to hold closer tolerances in the chemical composition.

An alloy containing, for instance, 3% magnesium and 2½% thorium, was prepared by such melting methods as just outlined, and in the cast condition, showed a Rockwell F. hardness 5 of 55. The material could be readily swaged and after a reduction of 30% increased in hardness to 94 F. The electrical conductivity of a material of such composition was 22.4% International annealed copper standard.

10 The superior qualities of alloys described by the present invention for electrical purposes, are illustrated by the following examples: A comparison test was conducted, wherein contacts of similar physical dimensions were tested on a 15 resistive inductive circuit at 470 cycles per minute and wherein the current flowing in the circuit was increased periodically to obtain the definite current values of alloys in the nature described above, in comparison with contact materials in the prior art. The amount of material transfer of one contact to the other was also used as a method of comparison.

20 Contacts of the following compositions, when operated under the above stated conditions, gave 25 outstanding performances compared to the alloys of the prior art, some of which are given for comparison:

| Contract material                                | Limiting current | Height of material transfer                                    |
|--------------------------------------------------|------------------|----------------------------------------------------------------|
| Alloy containing 3% Mg, 2.5% Th, and balance Ag. | 19               | .003 on the positive contact.<br>.004 on the negative contact. |
| 35 Fine silver.                                  | 12               | .010.                                                          |
| Coin silver.                                     | 11               | .011.                                                          |

The final contact resistance on these new and improved alloys, the composition of which are 40 given above, did not substantially exceed the values obtained for fine silver, under identical test conditions. The alloy containing, for instance, 3% magnesium and 2½% thorium, showed a contact resistance of .39 milliohms, 45 after the test.

It will be noted from the above test results that the metallic transfer, due to the operation of these contacts, is considerably smaller than on

fine silver. Also, this reduction in transfer has been obtained in spite of the fact that the new alloys were operated at much higher current values, and therefore under much more severe transfer producing conditions. It should also be 5 noted that the limiting current, that is, the current at which the contacts tends to weld together, is considerably higher than that of fine silver, the value for fine silver being 12 amps., and that for the improved alloy, 19 amps.

The alloys of the present invention have been found useful for a large number of electrical contact applications, such as, for instance, sensitive direct current relays, over-load cutouts, voltage regulators, indicating and recording 15 gaugers, thermostatic controls and the like.

Other uses of the new alloy are in the form of silverware, such as is used for table ware, industrial applications, jewelry purposes and the like.

The alloy of the present invention has also a 20 commercial advantage because the addition of magnesium in the percentage contemplated, provides a material of lower specific gravity and therefore it is possible to produce a larger number of finished products per unit weight of material.

While the present invention as to its objects and advantages has been described herein, as carried out in specific embodiments thereof, it is not desired to be limited thereby, but it is intended to cover the invention broadly, within the spirit and scope of the appended claims.

What is claimed is:

1. An alloy comprising .05 to 15% magnesium, .005 to 10% thorium, and the entire balance, 35 substantially all silver.

2. An alloy of .05 to 8% magnesium, .005 to 10% thorium, and the entire balance substantially all silver.

3. An alloy of 1 to 4% magnesium, .005 to 40 10% thorium, and the entire balance substantially all silver.

4. An alloy of 1 to 4% magnesium, .1 to 3% thorium, and the balance substantially all silver.

45  
FRANZ R. HENSEL.  
KENNETH L. EMMERT.  
JAMES W. WIGGS.